# EUROPEAN PATENT SPECIFICATION

(11) **EP 3 265 318 B1**
(45) Date of publication and mention of the grant of the patent: **02.10.2019**
(21) Application number: 15903176.4
(22) Date of filing: 28.08.2015
(51) Int. Cl.: B41J 5/50, C09D 129/04, D21H 19/20, B41M 5/52

(54) **PRIMER COMPOSITIONS**
GRUNDIERUNGSZUSAMMENSETZUNGEN
COMPOSITIONS DE COUCHE PRIMAIRE

(43) Date of publication of application: 10.01.2018
(73) Proprietor: Hewlett-Packard Development Company, L.P., Spring TX 77389 (US)
(72) Inventor: NIU, Bor-Jiunn, San Diego, California 92127-1899 (US); CHEN, Tao, San Diego, California 92127-1899 (US)
(74) Representative: Beccarelli, Sandra Béatrice Yvonne
(86) International application number: PCT/US2015/047447
(87) International publication number: WO 2017/039585

(56) References cited:
- WO-A1-2011/014199
- WO-A1-2015/116095
- US-A- 5 084 492
- US-A- 5 102 856
- US-A1- 2003 021 962
- US-A1- 2006 014 014
- US-A1- 2014 212 591
- US-A1- 2014 212 591

## Description

### BACKGROUND

There are several reasons that inkjet printing has become a popular way of recording images on various media surfaces, particularly paper. Some of these reasons include low printer noise, variable content recording, capability of high speed recording, and multi-color recording. Additionally, these advantages can be obtained at a relatively low price to consumers. Though there has been great improvement in inkjet printing, accompanying this improvement are increased demands by consumers in this area, e.g., higher speeds, higher resolution, full color image formation, increased stability, etc. Additionally, inkjet printing is becoming more prevalent in high speed commercial printing markets, competing with more laborious offset and gravure printing technologies. Coated media typically used for these more conventional types of printing, e.g., offset or gravure printing, can perform somewhat acceptably on high speed inkjet printing devices, but these types of media are not always acceptable for inkjet technology as it relates to image quality, gloss, abrasion resistance, and other similar properties.

### BRIEF DESCRIPTION OF THE DRAWINGS

Additional features and advantages of the disclosure will be apparent from the detailed description which follows, taken in conjunction with the accompanying drawings, which together illustrate, by way of example, features of the present technology.
FIG. 1 illustrates a method of coating a media substrate in accordance with an example of the present technology;
FIG. 2 shows a cross-sectional view of a coated media substrate in accordance with an example of the present technology; and
FIG. 3 shows a cross-sectional view of a coated media substrate in accordance with an example of the present technology.

Reference will now be made to several examples that are illustrated herein, and specific language will be used herein to describe the same. It will nevertheless be understood that no limitation of the scope of the disclosure is thereby intended.

### DETAILED DESCRIPTION

**The** present disclosure is drawn to primer compositions. In some examples, the primer compositions can be ink-receiving primer compositions, in that the primer compositions can be used to form coatings for receiving inks such as inkjet inks. The primer compositions can be applied to a substrate to form an ink-receiving layer on the substrate before printing inkjet ink over or onto the primer layer. In one example, a primer composition can be applied to offset coated paper. Typically, offset coated papers are significantly different from paper specifically designed for inkjet printing. Commercial offset paper often includes a smooth, nonporous surface coating that is difficult to penetrate by aqueous liquids. In many cases, offset coatings include inorganic pigments such as calcium carbonate and clay, as well as hydrophobic polymers that interact poorly with water-based inks. Polymers used in offset media can also sometimes include latex binders, polystyrenes, polyolefins (polypropylene, polyethylene, polybutadiene), polyesters (PET), polyacrylates, polymethacrylates, poly (maleic anhydride), and/or others. As a result of the hydrophobic and nonporous properties of offset media, water-based inks printed on offset media often have poor image quality, dry very slowly (sometimes taking more than 24 hours), and have poor durability after drying.

The primer compositions described herein can be applied to a media substrate, such as an offset media substrate as described above, to improve the ability of the substrate to receive water-based inks. For example, a primer composition can be coated on a media substrate to improve the durability of images printed with water-based inks. In one example, a media substrate that is normally less suitable for printing with water-based inks, such as offset media, can be coated with the primer composition prior to printing. This coated media substrate can interact with water-based inks and provide a printed image with good durability after the ink dries on the coated media substrate.

In further detail, the primer composition can include a water soluble polymeric binder, e.g., partially water soluble (at least 5%), mostly water soluble (at least 50%), or fully water soluble (at least 99%) in the primer composition. Water soluble polymers can interact better with water-based inks compared to the hydrophobic coatings of offset media. However, many types of water-soluble polymeric binder exhibit poor dry smearfastness immediately after printing due to poor wet film strength. For example, starches, cellulose, polyethylene oxide, and polyvinylpyrrolidone (PVP) are examples of water-soluble polymers that can have poor dry smearfastness when used in primers on offset media.

Poor dry smearfastness immediately after printing can be problematic because the printed image can be easily smeared if the image is rubbed or otherwise disturbed soon after printing. For example, when using an HP high speed Web Press@, the printing is a continuous process and the paper is rewound as a roll after printing. The image or text printed on the paper can be smeared when the paper is rewound if the dry durability is poor. Prior solutions to this problem have included reducing the printing speed, increasing drying temperature, or increasing the drying zone. Several disadvantages are associated with these solutions, however. For example, increasing the drying time requires reducing the production rate, which increases the cost or time cost of printing. Harsh drying conditions can cause increased paper cockle. Increasing the size of the drying zone makes the printing system occupy a larger space, which increases the total cost or space cost of printing.

Surprisingly, certain primer compositions including polyvinyl alcohols and other components have been found to provide much better dry smearfastness immediately after printing. Thus, the primer composition can include polyvinyl alcohol as the water soluble polymeric binder. In addition to the polyvinyl alcohol, the primer composition can include a cationic salt. Thus, the hydroxyl groups of the polyvinyl alcohol can interact with the cationic salt to form a complex-like structure. This structure can result in enhanced wet film strength of the primer layer and the ink printed on top of the primer layer. When inkjet ink is printed on top of the primer, the ink can have improved instant dry smearfastness.

Although primer compositions including polyvinyl alcohols can provide desirable dry smearfastness, it is difficult to achieve both dry smearfastness and wet smearfastness at the same time. Poor wet smearfastness can cause poor mechability because the printed substrate can often be rewound before the primer layer and image are completely dry. Mixtures of different water soluble polymeric binders can be used to adjust the dry smearfastness and wet smearfastness of the primer composition. However, many mixtures of water soluble polymeric binders are unable to provide both good dry smearfastness and good wet smearfastness. For example, mixtures of polyvinyl alcohol with common starch, polyvinyl pyrrolidone, or polyethylene oxide can in some cases provide good dry smearfastness or good wet smearfastness, but not both at the same time. However, certain primer compositions including a mixture of polyvinyl alcohol, starch nanoparticles, and a polymer latex dispersion have been found to provide better dry smearfastness and wet smearfastness at the same time.

The primer composition can be used on offset paper in a continuous printing system such as the HP high speed Web Press@ mentioned above. In some cases, a more immediate or instant dry and wet smearfastness of the printed image can be such that no smearing occurs when the printed paper is rewound into a roll after printing. Because the printed image does not need extra time to dry before rewinding the paper, the press can run at a high speed in some examples. These advantages can be obtained without compromising print quality.

With this description in mind, in some examples, the present technology provides primer compositions.

The primer composition comprises:
a) 5 wt% to 70 wt% of a binder that includes1 wt% to 40 wt% polyvinyl alcohol, 1 wt% to 20 wt% starch nanoparticles having an average diameter from 1 nm to 1 µm and 10 wt% to 70 wt% polymer latex dispersion;
b) 1 wt% to 20 wt% of a wax;
c) 10 wt% to 50 wt% of a cationic salt; and
d) water,
wherein components (a) to (c) are present in an amount of all dry components of the primer composition.
In some examples, the primer composition can also include other additives such as surfactants. It is notable that when the water and other volatiles evaporate off, the weight percentage of the various solids in the composition increase, i.e. in the ink-receiving primer layer discussed hereinafter.

The polyvinyl alcohol, starch nanoparticles, and polymer latex dispersion can act as a binder in the primer composition. Generally, the amount of these ingredients can be sufficient to act as a binder to bind the remaining ingredients of the primer composition to the substrate. In some examples, the binder content of the primer composition can be within a range such that there is sufficient binder to bind the other ingredients of the primer to the substrate, but not so much that the ink-receiving properties of the primer are compromised. As an example, too much binder can, in some cases, make the primer layer less porous and negatively impact the solution stability of the primer. This can interfere with the interaction between the primer layer and water-based inks. The total amount of binder present in the primer composition is from 5 wt% to 70 wt%. In other examples, the total amount of binder can be from 5 wt% to 50 wt%, 10 wt% to 30 wt%, or 10 wt% to 20 wt%.

In further detail, the primer composition includes polyvinyl alcohol in an amount from 1 wt% to 40 wt%, 2 wt% to 30 wt%, or 5 wt% to 20 wt%, based on the weight of all dry components of the primer composition.

The type of polyvinyl alcohol is not particularly limited with respect to the molecular weight and degree of hydrolysis of the polyvinyl alcohol. However, in some examples, the polyvinyl alcohol can have a weight-average molecular weight from 1,000 M_{w} to 300,000 M_{w}. In further examples, the polyvinyl alcohol can have an average molecular weight from about 20,000 M_{w} to about 250,000 M_{w}. In more specific examples, the polyvinyl alcohol can have an average molecular weight from about 27,000 M_{w} to about 205,000 M_{w}. The degree of hydrolysis of the polyvinyl alcohol can be from about 75 mol% to about 100 mol%. In certain examples, the degree of hydrolysis can be from about 86 mol% to about 100 mol%. It is believed that the hydroxyl groups on the polyvinyl alcohol can interact with the cationic salt in the primer composition to form a complex-like structure, which improves the instant smearfastness of printed images on a primer coated substrate. Non-limiting examples of polyvinyl alcohols that can be used in the primer composition include Poval® 3-88 (Kuraray America, Inc.) (14,000 M_{w}, 86.7-88.7 mol% hydrolysis); Poval® 4-88 (Kuraray America, Inc.) (31,000 M_{w}, 86.7-88.7 mol% hydrolysis); Poval® 4-98 (Kuraray America, Inc.) (27,000 M_{w}, 98-98.8 mol% hydrolysis); Poval® 5-88 (Kuraray America, Inc.) (37,000 M_{w}, 86.7-88.7 mol% hydrolysis); Poval® 8-88 (Kuraray America, Inc.) (67,000 M_{w}, 86.7-88.7 mol% hydrolysis); Poval® 13-88 (Kuraray America, Inc.) (86.7-88.7 mol% hydrolysis); Poval® 18-88 (Kuraray America, Inc.) (130,000 M_{w}, 86.7-88.7 mol% hydrolysis); Poval® 23-88 (Kuraray America, Inc.) (150,000 M_{w}, 86.7-88.7 mol% hydrolysis); Poval® 26-88 (Kuraray America, Inc.) (160,000 M_{w}, 86.7-88.7 mol% hydrolysis); and Poval® 40-88 (Kuraray America, Inc.) (205,000 M_{w}, 86.7-88.7 mol% hydrolysis).

The polyvinyl alcohol can in some cases be a mixture of two or more types of polyvinyl alcohol. In such examples, the total amount of the polyvinyl alcohols can be from 1 wt% to 40 wt%, 2 wt% to 30 wt%, 5 wt% to 20 wt%, based on the weight of all dry components of the primer composition. Whatever range is considered, it is understood that the range relates to total concentrations of polyvinyl alcohol, whether there be one, two, three, etc., specific polyvinyl alcohol species present. In one example, the primer composition can include a mixture of two types of polyvinyl alcohol having different molecular weights.

In addition to the polyvinyl alcohol, the binder can include starch nanoparticles. Starch is a carbohydrate consisting of linear or branched polysaccharide chains. Starch is often available in granular form, with granules having an average diameter of 10 µm to 100 µm or larger. Starch nanoparticles are different from this common form of starch in that the starch nanoparticles have a smaller, nano-sized average diameter. Starch nanoparticles have an average diameter from 1 nm to 1 µm. The starch nanoparticles used in the binder for the present primer compositions have an average diameter within this range of 1 nm to 1 µm. In some examples, the starch nanoparticles can have an average diameter from 10 nm to 500 nm, 20 nm to 200 nm, or 50 nm to 150 nm.

Non-limiting examples of suitable starch nanoparticles for use in the present primer compositions include Ecosphere® 2202D, 2260, 2330 and 2326 (EcoSynthetix Inc.). These starch nanoparticles are cross-linked starch with a nanoparticle structure, and can yield better durability than traditional starches that are non-crosslinked polymers. In some examples, the primer composition can include starch nanoparticles in an amount from 1 wt% to 20 wt%, 1 wt% to 10 wt%, or 2 wt% to 5 wt% based on the weight of all dry components of the primer composition.

**The** primer composition further includes a polymer latex dispersion. The polymer latex dispersion can include latex particles suspended in water or an aqueous system. In some examples, the latex particles is present in an amount from about 10 wt% to about 70 wt% based on the weight of all dry components of the primer composition. In further examples, the latex particles can be present in an amount from 20 wt% to 60 wt% based on the weight of all dry components of the primer composition. Additionally, the primer composition can be predominantly (greater than 50 wt% by dry weight) made up of the latex particles, the polyvinyl alcohol, the starch nanoparticles, wax, and the cationic salt. In one example, the polyvinyl alcohol, starch nanoparticles, polymer latex dispersion, wax, and cationic salt, can make up at least 80 wt% of all dry ingredients in the primer composition.

The latex particles can be used to improve the film strength of the primer layer. In one example, the glass transition temperature (Tg) of the latex can be from 0°C to 100°C. The latex polymer can be anionic, nonionic, or cationic. In some examples, the latex particles can be cationic latex particles.

In other examples, the latex particles can be made of polymers and copolymers including acrylic polymers or copolymers, vinyl acetate polymers or copolymers, polyester polymers or copolymers, vinylidene chloride polymers or copolymers, butadiene polymers or copolymers, styrene-butadiene polymers or copolymers, acrylonitrile-butadiene polymers or copolymers. In another example, the latex particles can include a vinyl acetate-based polymer, an acrylic polymer, a styrene polymer, a styrene-butadiene (SBR)-based polymer, a polyester-based polymer, a vinyl chloride-based polymer, an acid-based polymer, or the like. In one aspect, the latex particles can be a polymer or a copolymer including acrylic polymers, vinyl-acrylic copolymers and acrylic-polyurethane copolymers. In another aspect, the latex particles can be cationic acrylate latex. In one specific aspect, the latex can be a vinyl acetate polymer. In another specific aspect, the latex can be a SBR polymer.

Generally, the latex particles can have a weight average molecular weight (M_{w}) of 5,000 M_{w} to 500,000 M_{w}. In one example, the latex particles can range from 150,000 M_{w} to 300,000 M_{w}. In some examples, the average particle diameter of the latex particles can be from 10 nm to 1 µm and, as other examples, from 10 nm to 500 nm, and in yet other examples, from 50 nm to 250 nm. The particle size distribution of the latex is not particularly limited, and either latex having a broad particle size distribution or latex having a mono-dispersed particle size distribution may be used. It is also possible to use two or more kinds of polymer fine particles each having a mono-dispersed particle size distribution in combination

In some cases, the primer composition can include additional binders. Non-limiting examples of such binders include cellulose, polyethylene oxide, polyvinyl pyrrolidone, and others. The additional binders can also be mixtures of two or more water soluble polymeric binders. In some examples, if additional binders are present then the additional binders can be present in a smaller amount than the combined polyvinyl alcohol, starch nanoparticles, and polymer latex dispersion. In further examples, the combined polyvinyl alcohol, starch nanoparticles, and polymer latex dispersion can make up at least 10 wt% by dry weight of all binders present in the primer composition. In still further examples, the combined polyvinyl alcohol, starch nanoparticles, and polymer latex dispersion can make up at least 80 wt% by dry weight of all binders present in the primer composition. In a specific example, the primer composition can be substantially free of any binder other than the polyvinyl alcohol, starch nanoparticles, and polymer latex dispersion.

The primer composition also includes a wax. In some examples, the wax can act as a slip aid to contribute to abrasion resistance and coefficient of friction (COF) reduction. Suitable waxes can include particles of a synthetic wax, natural wax, combinations of a synthetic wax and a natural wax, combinations of two or more different synthetic waxes, or combinations of two or more different natural waxes, for example. In some examples, the synthetic wax can include polyethylene, polypropylene, polybutadiene, polytetrafluoroethylene, polyvinylfluoride, polyvinyldiene fluoride, polychlorotrifluoroethylene, perfluoroalkoxy polymer, perfluoropolyether, polyurethane, polyethylenechlorotrifluoroethylene, polyethylene-vinyl acetate, epoxy resin, silicone resin, polyamide resin, polyamide, or polyester resin. In some examples, the natural wax can include carnauba wax, paraffin wax, montan wax, candelilla wax, ouricury wax, sufarcane wax, retamo wax, or beeswax. In one example, the wax can be a polyethylene wax, such as a high density polyethylene wax. Commercially available slip aids that can be used include Michemshield® 29235 (Michelman, Inc.), Ultralube® E846 (Keim-Additec Surface GmbH), and Ultralube® D-806 (Keim-Additec Surface GmbH), for example. In some examples, a wax is present in the primer composition at an amount of 1 wt% to 20 wt% of all dry ingredients in the primer composition. In other examples, the wax can be present in an amount of 5 wt% to 15 wt% of all dry ingredients in the primer composition

The primer composition also includes a cationic salt. The cationic salt can be present in an amount sufficient to immobilize pigment colorants in the ink to be printed over the primer and to yield good image quality. In some examples, the primer composition can include the cationic salt in an amount from 10 wt% to 50 wt%, 10 wt% to 40 wt%, 15 wt% to 30 wt%, or 20 wt% to 30 wt% based on the weight of all dry components of the primer composition.

The cationic salt can include a metal cation. In some examples, the metal cation can be sodium, calcium, copper, nickel, magnesium, zinc, barium, iron, aluminum, chromium, or other metal. The cationic salt can also include an anion. In some examples, the anion can be fluoride, chloride, iodide, bromide, nitrate, chlorate, acetate, or RCOO⁻ where R is hydrogen or any low molecular weight hydrocarbon chain, e.g., C1 to C12. In a more specific example, the anion can be a carboxylate derived from a saturated aliphatic monocarboxylic acid having 1 to 6 carbon atoms or a carbocyclic monocarboxylic acid having 7 to 11 carbon atoms. Examples of saturated aliphatic monocarboxylic acid having 1 to 6 carbon atoms may include formic acid, acetic acid, propionic acid, butyric acid, isobutyric acid, valeric acid, isovaleric acid, pivalic acid, and/or hexanoic acid. In some cases, the cationic salt can be a polyvalent metal salt made up of a divalent or higher polyvalent metallic ion and an anion. In certain examples, the cationic salt can include calcium chloride, calcium nitrate, magnesium nitrate, magnesium acetate, and/or zinc acetate. In one aspect, the cationic salt can include calcium chloride or calcium nitrate (CaCl₂ or Ca(NO₃)₂). In one additional specific aspect, the cationic salt can include calcium chloride (CaCl₂). The cationic salt can also be a mixture of two or more different cationic salts. In such examples, the total amount of the mixture of cationic salts can be 10 wt% to 50 wt%, 10 wt% to 40 wt%, 15 wt% to 30 wt%, or 20 wt% to 30 wt% based on the weight of all dry components of the primer composition. Whatever range is considered, it is understood that the range relates to total concentrations of salts, whether there be one, two, three, etc., specific salt species present.

Many coating compositions for inkjet printing include inorganic pigments to improve the absorption properties of the coating. Such inorganic pigments can include, for example, clays such as kaolin clay or calcined clay, ground calcium carbonate, precipitated calcium carbonate, barium sulfate, titanium dioxide, silica, aluminum trihydrate, aluminum oxide, boehmite, or combinations thereof. However, in some examples, the present primer composition can be substantially devoid of inorganic pigments. In other examples, the primer composition can include an inorganic pigment. In some examples, the primer composition can include an inorganic pigment in an amount of about 5 wt% or less of all dry components of the primer composition. Thus, the primer composition can include a relatively small amount of inorganic pigment, such as less than 5 wt%. In certain examples, the primer composition can be acidic and can include an inorganic pigment that is compatible with acid, such as a clay.

The primer composition can also include other coating additives such as surfactants, rheology modifiers, defoamers, optical brighteners, biocides, pH controlling agents, dyes, and other additives for further enhancing the properties of the primer composition. The total amount of such optional coating additives can be present, individually, in the range of 0.01 wt% to 5 wt% of all dry ingredients of the primer composition.

The present technology also extends to methods of coating a media substrate. FIG. 1 provides an exemplary method of coating a media substrate 100. The method includes applying 110 a primer composition to a media substrate, wherein the primer composition includes from 5 wt% to 70 wt% binder including polyvinyl alcohol, starch nanoparticles, and a polymer latex dispersion. The primer composition further includes a wax, a cationic salt and water.

The primer composition used in the method can have any of the ingredients in the amounts described above with respect to the primer composition. In a particular example, the method can include applying a primer composition that includes the polyvinyl alcohol in an amount from 1 wt% to 40 wt% of all dry ingredients in the primer composition, starch nanoparticles in an amount from 1 wt% to 20 wt%, and a polymer latex dispersion in an amount from 20 wt% to 70 wt% of all dry ingredients in the primer composition. In a further example, the method can include applying a primer composition in which polyvinyl alcohol, starch nanoparticles, polymer latex dispersion, wax and cationic salt make up at least 80 wt% of all dry ingredients in the primer composition. In yet another example, the method can include applying a primer composition that is substantially devoid of inorganic pigments. In another example, the method can include applying a primer composition that includes an inorganic pigment in an amount of about 5 wt% or less of all dry components of the primer composition.

The composition can be applied to the substrate by any of a number of coating methods. In accordance with examples of the present disclosure, the substrate can be coated by spray coating, dip coating, cascade coating, roll coating, gravure coating, curtain coating, air knife coating, cast coating, Meyer rod coating, blade coating, film coating, metered size press coating, puddle size press coating, calender stack, and/or by using other known coating techniques. The thickness selected for the coating layer can vary. In one example, the primer composition can be applied at a dry coat weight from 0.1 gsm to 20 gsm. In another example, the primer composition can be applied to the substrate at a dry coat weight from 0.3 gsm to 10 gsm. In another example, the primer composition can be applied to the substrate at a dry coat weight from 0.3 gsm to 5 gsm. In another example, the primer composition can be applied to the substrate at a dry coat weight from 0.3 gsm to 1 gsm.

The method of coating the media substrate can further include allowing a sufficient time for the primer layer to dry before printing ink on the primer layer. The primer layer can be dried with infrared lamp, hot air and combination thereof. The primer layer can retain from about 0.01 wt% to about 10 wt% water, based on the total weight of the coating, when the coating is dry enough to print on. In some examples, the coating can have from about 1 wt% to about 6 wt% water remaining when an image is printed on the coated substrate. Thus, it is understood that the "dry coat weight" described herein refers to dry components, even if some water remains behind in the final formulation coating.

Ink can be printed on the primer layer. Printing can occur when the primer layer is partially dry or fully dry (i.e. dry to the touch but still may include some residual water). In some cases, the ink can be a water-based ink such as a water-based inkjet ink. Inkjet inks generally include a colorant dispersed or dissolved in an ink vehicle. As used herein, "liquid vehicle" or "ink vehicle" refers to the liquid fluid in which a colorant is placed to form an ink. Ink vehicles are well known in the art, and a wide variety of ink vehicles may be used with the systems and methods of the present disclosure. Such ink vehicles may include a mixture of a variety of different agents, including, surfactants, solvents, co-solvents, anti-kogation agents, buffers, biocides, sequestering agents, viscosity modifiers, surface-active agents, water, etc. Though not part of the liquid vehicle per se, in addition to the colorants, the liquid vehicle can carry solid additives such as polymers, latexes, UV curable materials, plasticizers, etc.

Generally the colorant discussed herein can include a pigment and/or dye. As used herein, "dye" refers to compounds or molecules that impart color to an ink vehicle. As such, dye includes molecules and compounds that absorb electromagnetic radiation or certain wavelengths thereof. For example, dyes include those that fluoresce and those that absorb certain wavelengths of visible light. In most instances, dyes are water soluble. Furthermore, as used herein, "pigment" generally includes pigment colorants, magnetic particles, aluminas, silicas, and/or other ceramics, organo-metallics or other opaque particles. In one example, the colorant can be a pigment.

Consistent with the formulation of this disclosure, various other additives may be employed to enhance the properties of the ink composition for specific applications. Examples of these additives are those added to inhibit the growth of harmful microorganisms. These additives may be biocides, fungicides, and other microbial agents, which are routinely used in ink formulations. Examples of suitable microbial agents include, but are not limited to, NUOSEPT® (Nudex, Inc.), UCARCIDE™ (Union carbide Corp.), VANCIDE® (R.T. Vanderbilt Co.), PROXEL® (ICI America), ACTICIDE® (Thor Specialties Inc.) and combinations thereof.

The present technology also extends to coated media substrates. The media substrate can include a variety of types of base substrate, including paper media, nonporous media, swellable media, microporous media, photobase media, offset media, coated media, uncoated media, and other types of media including plastics, vinyl media, fabrics, woven substrate, etc. In certain examples, the substrate can be a swellable media, a microporous media, or an offset media. The primer composition according to the present technology can be especially useful for coating offset media, which typically has a very small pore diameter (often referred to a nonporous) and hydrophobic surface that does not interact well with water based inks.

In one example, a coated media substrate according to the present technology can include a media substrate and a primer layer coated on a surface of the media substrate. The primer layer can include a binder having polyvinyl alcohol, starch nanoparticles, and a polymer latex dispersion. The primer layer can also include a wax and a cationic salt.

FIG. 2 shows an example of a coated media substrate 200. A base substrate 210 is coated with a primer layer 220. On top of the primer layer, ink jet ink 230 can be printed to form a printed image. The image can have improved instant dry smearfastness after printing.

FIG. 3 shows another example of a coated media substrate 300. In this example, the base substrate 310 has a primer layer 320 coated on both sides of the base substrate. Ink jet ink 330 is used to print images one or on both sides of the coated substrate. Thus, the coated media substrate can be used for double sided printing. Although not shown in the figures, the base substrate can also include its own coating, such as the hydrophobic coating on offset paper. Certain coatings (or pre-coatings) described herein can often already be present as part of a substrate, and these coatings are not the same as the primer layer primarily discussed in the context of the present disclosure. Offset media or photobase, for example, already include coatings on one or both side of a substrate material (and thus are considered to be part of the base substrate). The primer compositions of the present disclosure, conversely, are those which are overcoated with respect to the pre-applied coatings, or alternatively, to substrates that are not already pre-coated. Such coatings, i.e. the pre-coating and/or the primer compositions of the present disclosure, can be present on either one side of a media substrate or both.

The primer layer on the coated substrate can be formed by applying the primer compositions disclosed herein using any of the methods disclosed herein. As such, the primer layer can include any of the additional ingredients in any of the amounts disclosed for the primer compositions described herein. In a specific example, the primer layer can include the polymer latex dispersion in an amount from 10 wt% to 70 wt% of all dry components of the primer layer. Additionally, the polyvinyl alcohol, starch nanoparticles, polymer latex dispersion, wax, and cationic salt can make up at least 80 wt% of all dry components of the primer layer.

In yet another example of the present technology, a printing system can include an inkjet ink and a coated media substrate as described above. The coated media substrate can include a media substrate and a primer layer coated on a surface of the media substrate. The primer layer can include a polyvinyl alcohol, starch nanoparticles, a polymer latex dispersion, a wax and a cationic salt.

It is noted that, as used in this specification and the appended claims, the singular forms "a," "an," and "the" include plural referents unless the content clearly dictates otherwise.

"Substrate" or "media substrate" includes any base material that can be coated in accordance with examples of the present disclosure, such as film base substrates, polymer substrates, conventional paper substrates, photobase substrates, offset media substrates, and the like. Further, pre-coated and film coated substrates can be considered a "substrate" that can be further coated in accordance with examples of the present disclosure.

"Slip aid" refers to materials that can be added to coating compositions herein to provide abrasion resistance to coatings of the present disclosure.

"Instant dry smearfastness" refers to the ability of a printed image to resist smearing when rubbed with a dry instrument such as a finger or a Rubber Eraser Tool, immediately after printing or within a short time of being printed. The short time can be, for example, from 1 second to 30 seconds, from 1 second to 20 seconds, or from 5 seconds to 10 seconds. In some cases, the short time can be the time required for a printed image to travel from the inkjet printer to a rewinding roll. In one example, a printed image on an HP T230 Web Press@ takes from 5 seconds to 10 seconds to reach the rewinder after being printed.

"Instant wet smearfastness" refers to the ability of a printed image to resist smearing when rubbed with a wet instrument such as a wet finger immediately after printing or within a short time of being printed. The short time can be, for example, from 1 second to 30 seconds, from 1 second to 20 seconds, or from 5 seconds to 10 seconds. In some cases, the short time can be the time required for a printed image to travel from the inkjet printer to a rewinding roll. In one example, a printed image on an HP T230 Web Press@ takes from 5 seconds to 10 seconds to reach the rewinder after being printed.

"Instant mechability" refers to the instant dry and wet smearfastness and the scratch resistance of a sample after printing, drying, and reaching the rewinding station.

When referring to "high speed" as it related to a digital printing press, presses such as the HP T230 Web Press@ or the HP T350 Web Press@ exhibit printing speeds that are commensurate of what is considered to be "high speed." For example, the HP T350 Web Press@ can print text and/or other images on media at a rate of 400 feet per minute. This capability would be considered high speed. In another example, and more generally, printing at 100 feet per minute would also be considered high speed.

As used herein, the term "about" is used to provide flexibility to a numerical range endpoint by providing that a given value may be "a little above" or "a little below" the endpoint. The degree of flexibility of this term can be dictated by the particular variable and can be determined based on experience and the associated description herein.

As used herein, a plurality of items, structural elements, compositional elements, and/or materials may be presented in a common list for convenience. However, these lists should be construed as though each member of the list is individually identified as a separate and unique member. Thus, no individual member of such list should be construed as a *de facto* equivalent of any other member of the same list solely based on their presentation in a common group without indications to the contrary.

Concentrations, dimensions, amounts, and other numerical data may be presented herein in a range format. It is to be understood that such range format is used merely for convenience and brevity and should be interpreted flexibly to include not only the numerical values explicitly recited as the limits of the range, but also to include all the individual numerical values or sub-ranges encompassed within that range as if each numerical value and sub-range is explicitly recited. For example, a weight ratio range of about 1 wt% to about 20 wt% should be interpreted to include not only the explicitly recited limits of 1 wt% and about 20 wt%, but also to include individual weights such as 2 wt%, 11 wt%, 14 wt%, and sub-ranges such as 10 wt% to 20 wt%, 5 wt% to 15 wt%, etc.

As a further note, in the present disclosure, it is noted that when discussing the coated media substrate, the method of coating a substrate, or the primer compositions herein, each of these discussions can be considered applicable to each of these examples, whether or not they are explicitly discussed in the context of that example. Thus, for example, in discussing details about the coated media substrate *per se*, such discussion also refers to the methods and primer compositions described herein, and *vice versa.*

The following examples illustrate some of the primer compositions, coated media substrates, systems, and methods that are presently known. However, it is to be understood that the following are only exemplary or illustrative of the application of the principles of the present compositions, systems, and methods. Numerous modifications and alternative compositions, systems, and methods may be devised without departing from the spirit and scope of the present disclosure. The appended claims are intended to cover such modifications and arrangements. Thus, while the examples have been described above with particularity, the following provide further detail in connection with what are presently deemed to be the acceptable examples.

### EXAMPLES

Formulation Examples 1-9 were prepared according to Tables 1A and 1B. Examples 7-9 are examples prepared according to the present technology and Examples 1-6 are comparative examples.

**Table 1A**

| Example No. Ingredient Dry Wt% | 1 | 2 | 3 | 4 | 5 |
|---|---|---|---|---|---|
| Poval® 4-88 (polyvinyl alcohol) | 2 | - | 2 | 2 | 2 |
| Poval® 18-88 (polyvinyl alcohol) | 9 | 18 | 9 | 9 | 9 |
| Penford® Gum 280 (starch) | - | - | 4 | - | - |
| Ecosphere® 2202D (starch nanoparticles) | - | - | - | - | - |
| Polyvinyl pyrrolidone (30,000 M_{w}) | - | - | - | 4 | - |
| Polyox™ N750 (polyethylene oxide) | - | - | - | - | 4 |
| Litex® 9710 (carboxylated styrene-butadiene copolymer latex) | 50 | 45 | 48 | 48 | 48 |
| Ultralube® D-806 (polyethylene wax) | 11 | 10 | 10 | 10 | 10 |
| Calcium Chloride (cationic salt) | 27 | 26 | 26 | 26 | 26 |
| TEGO® Wet 510 (surfactant) | 1 | 1 | 1 | 1 | 1 |

**Table 1B**

| Example No. Ingredient Dry Wt% | 6 | 7 | 8 | 9 |
|---|---|---|---|---|
| Poval® 4-88 (polyvinyl alcohol) | - | - | 2 | - |
| Poval® 18-88 (polyvinyl alcohol) | - | 4 | 9 | 9 |
| Penford® Gum 280 (starch) | - | - | - | - |
| Ecosphere® 2202D (starch nanoparticles) | 11 | 9 | 4 | 4 |
| Polyvinyl pyrrolidone (30,000 M_{w}) | - | - | - | - |
| Polyox™ N750 (polyethylene oxide) | - | - | - | - |
| Litex® 9710 (carboxylated styrene-butadiene copolymer latex) | 50 | 50 | 48 | 50 |
| Ultralube® D-806 (polyethylene wax) | 11 | 10 | 10 | 10 |
| Calcium Chloride (cationic salt) | 27 | 26 | 26 | 26 |
| TEGO® Wet 510 (surfactant) | 1 | 1 | 1 | 1 |

| | | | | |
|---|---|---|---|---|
| Poval® (from Kuraray America, Inc.) Ultralube® (from Keim-Additec Surface GmbH) TEGO® (from Evonik Resource Efficiency GmbH) Ecosphere® (from EcoSynthetix Inc.) Litex® (from Synthomer LLC) Polyox™ (from Dow Chemical Company) Penford® Gum (from Penford Products Co.) | | | | |

The Example formulations 1-9 were coated onto Sterling® Ultra Gloss (Verso Corporation), 60# paper with 2 g/m² (gsm) of dry coating weight. Samples were printed with an HP CM8060 MFP Edgeline printer, from Hewlett-Packard Co., Palo Alto, CA, USA (HP), using HP A50 pigment inks (i.e. aqueous inkjet ink for digital inkjet printing). The printing process used involved 2 passes and six dry spin conditions to mimic high-speed, digital, web press inkjet printing. Dry and wet smearfastness refer to the ability of the printed image to resist appearance degradation upon rubbing or smearing the image by dry or wet finger. For the dry and wet finger smearfastness tests, a dry or wet finger was placed against a printed area, pushed with force of about 50 g/in², and drawn toward the tester. The finger was then released to check the tested area.

The results of the dry finger smearfastness test and wet finger smearfastness test are shown in Table 2. For the dry and wet finger smearfastness tests, the visual ranking is based on a 1 to 5 scale, with 1 being the worst and 5 being the best. A ranking equal to or greater than 3 is considered good and acceptable. A ranking below 3 is considered poor and not acceptable.

**Table 2: Visual Ranking of Performance**

| Example No. | Dry Finger Smearfastness | Wet Finger Smearfastness |
|---|---|---|
| 1 | 3.5 | 2.5 |
| 2 | 3.5 | 2.5 |
| 3 | 3 | 2.5 |
| 4 | 3.25 | 2.5 |
| 5 | 3.25 | 2.5 |
| 6 | 1.5 | 1.5 |
| 7 | 2.5 | 4 |
| 8 | 3.5 | 3 |
| 9 | 3.25 | 3 |

Examples 1-5 did not include starch nanoparticles. These examples did not provide sufficient wet finger smearfastness. Example 6 included starch nanoparticles, but no polyvinyl alcohol. This example showed very poor dry finger smearfastness and wet finger smearfastness. Examples 7-9 included both starch nanoparticles and polyvinyl alcohol (as well as latex particles). Example 7 provided excellent wet finger smearfastness but marginal dry finger smearfastness. Examples 8 and 9 both provided good dry finger smearfastness and wet finger smearfastness. Therefore, these examples show that, although neither starch nanoparticles nor polyvinyl alcohol can provide sufficient wet and dry smearfastness when used alone, the combination of these two binders, along with latex particles) unexpectedly provides good wet and dry smearfastness.

## Claims

1. A primer composition, comprising:
a) 5 wt% to 70 wt% of a binder including:
i) 1 wt% to 40 wt% polyvinyl alcohol
ii) 1 wt% to 20 wt% starch nanoparticles having an average diameter from 1 nm to 1 µm; and
iii) 10 wt% to 70 wt% polymer latex dispersion,
b) 1 wt% to 20 wt% of a wax;
c) 10 wt% to 50 wt% of a cationic salt; and
d) water,
wherein components (a) to (c) are present in an amount of all dry components of the primer composition.

2. The primer composition of claim 1, wherein the polymer latex dispersion is selected from an SBR-based latex dispersion, a cationic acrylate latex dispersion, a polyvinyl acetate latex dispersion, and combinations thereof.

3. The primer composition of claim 2, wherein the starch nanoparticles are crosslinked starch nanoparticles.

4. The primer composition of claim 1, wherein the cationic salt comprises a cation of a metal selected from the group consisting of sodium, calcium, copper, nickel, magnesium, zinc, barium, iron, aluminum and chromium.

5. The primer composition of claim 1, wherein the polyvinyl alcohol, starch nanoparticles, polymer latex dispersion, wax, and cationic salt make up at least 80 wt% of all dry components of the primer composition.

6. The primer composition of claim 1, wherein the polyvinyl alcohol is a mixture of two different polyvinyl alcohols with different weight-average molecular weights.

7. The primer composition of claim 1, wherein the primer composition further comprises an inorganic pigment in an amount of 5 wt% or less of all dry components of the primer composition.

8. A method of coating a media substrate, comprising applying a primer composition to a media substrate, wherein the primer composition comprises:
a) 5 wt% to 70 wt% of a binder including:
i) 1 wt% to 40 wt% polyvinyl alcohol
ii) 1 wt% to 20 wt% starch nanoparticles having an average diameter from 1 nm to 1 µm; and
iii) 10 wt% to 70 wt% polymer latex dispersion,
b) 1 wt% to 20 wt% of a wax;
c) 10 wt% to 50 wt% of a cationic salt; and
d) water,
wherein components (a) to (c) are present in an amount of all dry components of the primer composition.

9. The method of claim 8, wherein the polyvinyl alcohol, starch nanoparticles, polymer latex dispersion, wax, and cationic salt make up at least 80 wt% of all dry components of the primer composition.

10. The method of claim 8, wherein the starch nanoparticles are crosslinked starch nanoparticles.

11. A coated media substrate, comprising:
a media substrate; and
an ink-receiving primer layer coated on a surface of the media substrate, the primer layer comprising:
a) 5 wt% to 70 wt% of a binder including:
i) 1 wt% to 40 wt% polyvinyl alcohol
ii) 1 wt% to 20 wt% starch nanoparticles having an average diameter from 1 nm to 1 µm; and
iii) 10 wt% to 70 wt% polymer latex dispersion,
b) 1 wt% to 20 wt% of a wax;
c) 10 wt% to 50 wt% of a cationic salt; and
d) water,
wherein components (a) to (c) are present in an amount of all dry components of the primer composition.

12. The coated media substrate of claim 11, wherein the media substrate is a smooth, nonporous offset media substrate.

13. The coated media substrate of claim 11, wherein the starch nanoparticles are crosslinked starch nanoparticles, and wherein the polyvinyl alcohol, starch nanoparticles, polymer latex dispersion, wax, and cationic salt make up at least 80 wt% of all dry components of the primer layer.

## Patentansprüche

1. Grundierungszusammensetzung, die Folgendes umfasst:
a) 5 Gew.-% bis 70 Gew.-% eines Bindemittels, einschließlich:
i) 1 Gew.-% bis 40 Gew.-% Polyvinylalkohol
ii) 1 Gew.-% bis 20 Gew.-% Stärkenanopartikel mit einem mittleren Durchmesser von 1 nm bis 1 µm; und
iii) 10 Gew.-% bis 70 Gew.-% Polymerlatexdispersion,
b) 1 Gew.-% bis 20 Gew.-% eines Wachses;
c) 10 Gew.-% bis 50 Gew.-% eines kationischen Salzes; und
d) Wasser,
wobei Komponenten (a) bis (c) in einer Menge aller trockenen Komponenten der Grundierungszusammensetzung vorhanden sind.

2. Grundierungszusammensetzung nach Anspruch 1, wobei die Polymerlatexdispersion aus einer Latexdispersion auf *SBR*(*styrene-butadiene rubber-* Styrol-Butadien-Kautschuk)-Basis, einer kationischen Acrylatlatexdispersion, einer Polyvinylacetatlatexdispersion und Kombinationen davon ausgewählt ist.

3. Grundierungszusammensetzung nach Anspruch 2, wobei die Stärkenanopartikel vernetzte Stärkenanopartikel sind.

4. Grundierungszusammensetzung nach Anspruch 1, wobei das kationische Salz ein Kation eines Metalls, ausgewählt aus der Gruppe bestehend aus Natrium, Calcium, Kupfer, Nickel, Magnesium, Zink, Barium, Eisen, Aluminium und Chrom, umfasst.

5. Grundierungszusammensetzung nach Anspruch 1, wobei der Polyvinylalkohol, die Stärkenanopartikel, die Polymerlatexdispersion, das Wachs und das kationische Salz wenigstens 80 Gew.-% aller trockenen Komponenten der Grundierungszusammensetzung ausmachen.

6. Grundierungszusammensetzung nach Anspruch 1, wobei der Polyvinylalkohol eine Mischung aus zwei verschiedenen Polyvinylalkoholen mit verschiedenen gewichtsgemittelten Molekulargewichten ist.

7. Grundierungszusammensetzung nach Anspruch 1, wobei die Grundierungszusammensetzung ferner ein anorganisches Pigment in einer Menge von höchstens 5 Gew.-% aller trockenen Komponenten der Grundierungszusammensetzung umfasst.

8. Verfahren zum Beschichten eines Mediensubstrats, das ein Aufbringen einer Grundierungszusammensetzung auf ein Mediensubstrat umfasst, wobei die Grundierungszusammensetzung Folgendes umfasst:
a) 5 Gew.-% bis 70 Gew.-% eines Bindemittels, einschließlich:
i) 1 Gew.-% bis 40 Gew.-% Polyvinylalkohol
ii) 1 Gew.-% bis 20 Gew.-% Stärkenanopartikel mit einem mittleren Durchmesser von 1 nm bis 1 µm; und
iii) 10 Gew.-% bis 70 Gew.-% Polymerlatexdispersion,
b) 1 Gew.-% bis 20 Gew.-% eines Wachses;
c) 10 Gew.-% bis 50 Gew.-% eines kationischen Salzes; und
d) Wasser,
wobei Komponenten (a) bis (c) in einer Menge aller trockenen Komponenten der Grundierungszusammensetzung vorhanden sind.

9. Verfahren nach Anspruch 8, wobei der Polyvinylalkohol, die Stärkenanopartikel, die Polymerlatexdispersion, das Wachs und das kationische Salz wenigstens 80 Gew.-% aller trockenen Komponenten der Grundierungszusammensetzung ausmachen.

10. Verfahren nach Anspruch 8, wobei die Stärkenanopartikel vernetzte Stärkenanopartikel sind.

11. Beschichtetes Mediensubstrat, das Folgendes umfasst:
ein Mediensubstrat; und
eine tintenaufnehmende Grundierungsschicht, die auf eine Oberfläche des Mediensubstrats beschichtet ist, wobei die Grundierungsschicht Folgendes umfasst:
a) 5 Gew.-% bis 70 Gew.-% eines Bindemittels, einschließlich:
i) 1 Gew.-% bis 40 Gew.-% Polyvinylalkohol
ii) 1 Gew.-% bis 20 Gew.-% Stärkenanopartikel mit einem mittleren Durchmesser von 1 nm bis 1 µm; und
iii) 10 Gew.-% bis 70 Gew.-% Polymerlatexdispersion,
b) 1 Gew.-% bis 20 Gew.-% eines Wachses;
c) 10 Gew.-% bis 50 Gew.-% eines kationischen Salzes; und
d) Wasser,
wobei Komponenten (a) bis (c) in einer Menge aller trockenen Komponenten der Grundierungszusammensetzung vorhanden sind.

12. Beschichtetes Mediensubstrat nach Anspruch 11, wobei das Mediensubstrat ein glattes, nicht poröses Offset-Mediensubstrat ist.

13. Beschichtetes Mediensubstrat nach Anspruch 11, wobei die Stärkenanopartikel vernetzte Stärkenanopartikel sind, und wobei der Polyvinylalkohol, die Stärkenanopartikel, die Polymerlatexdispersion, das Wachs und das kationische Salz wenigstens 80 Gew.-% aller trockenen Komponenten der Grundierungsschicht ausmachen.

## Revendications

1. Composition de primaire comprenant :
a) 5% en poids à 70% en poids d'un liant comprenant :
i) 1% en poids à 40% en poids d'alcool polyvinylique
ii) 1% en poids à 20% en poids de nanoparticules d'amidon ayant un diamètre moyen compris entre 1 nm et 1 µm ; et
iii) 10% en poids à 70% en poids de dispersion de latex de polymère,
b) 1% en poids à 20% en poids d'une cire ;
c) 10% en poids à 50% en poids d'un sel cationique ; et
d) de l'eau,
dans lequel les composants (a) à (c) sont présents en une quantité de tous les composants secs de la composition de primaire.

2. Composition de primaire selon la revendication 1, dans laquelle la dispersion de latex de polymère est choisie parmi une dispersion de latex à base de SBR, une dispersion de latex d'acrylate cationique, une dispersion de latex d'acétate de polyvinyle et leurs combinaisons.

3. Composition de primaire selon la revendication 2, dans laquelle les nanoparticules d'amidon sont des nanoparticules d'amidon réticulé.

4. Composition de primaire selon la revendication 1, dans laquelle le sel cationique comprend un cation d'un métal choisi dans le groupe constitué par le sodium, le calcium, le cuivre, le nickel, le magnésium, le zinc, le baryum, le fer, l'aluminium et le chrome.

5. Composition de primaire selon la revendication 1, dans laquelle l'alcool polyvinylique, les nanoparticules d'amidon, la dispersion de latex de polymère, la cire et le sel cationique constituent au moins 80% en poids de tous les composants secs de la composition de primaire.

6. Composition de primaire selon la revendication 1, dans laquelle l'alcool polyvinylique est un mélange de deux alcools polyvinyliques différents ayant des poids moléculaires moyens de poids différents.

7. Composition de primaire selon la revendication 1, dans laquelle la composition de primaire comprend en outre un pigment inorganique en une quantité de 5% en poids ou moins de tous les composants secs de la composition de primaire.

8. Procédé de revêtement d'un substrat de support, consistant en l'application d'une composition de primaire à un substrat de support, dans lequel la composition de primaire comprend :
a) 5% en poids à 70% en poids d'un liant comprenant :
i) 1% en poids à 40% en poids d'alcool polyvinylique
ii) 1% en poids à 20% en poids de nanoparticules d'amidon ayant un diamètre moyen compris entre 1 nm et 1 µm ; et
iii) 10% en poids à 70% en poids de dispersion de latex de polymère,
b) 1% en poids à 20% en poids d'une cire ;
c) 10% en poids à 50% en poids d'un sel cationique ; et
d) de l'eau,
dans lequel les composants (a) à (c) sont présents en une quantité de tous les composants secs de la composition de primaire.

9. Procédé selon la revendication 8, dans lequel l'alcool polyvinylique, les nanoparticules d'amidon, la dispersion de latex de polymère, la cire et le sel cationique constituent au moins 80% en poids de tous les composants secs de la composition de primaire.

10. Procédé selon la revendication 8, dans lequel les nanoparticules d'amidon sont des nanoparticules d'amidon réticulé.

11. Un substrat de support revêtu, comprenant :
un substrat de support ; et
une couche de primaire réceptrice d'encre appliquée sur une surface du substrat, la couche de primaire comprenant :
a) 5% en poids à 70% en poids d'un liant comprenant :
i) 1% en poids à 40% en poids d'alcool polyvinylique
ii) 1% en poids à 20% en poids de nanoparticules d'amidon ayant un diamètre moyen compris entre 1 nm et 1 µm ; et
iii) 10% en poids à 70% en poids de dispersion de latex de polymère,
b) 1% en poids à 20% en poids d'une cire ;
c) 10% en poids à 50% en poids d'un sel cationique ; et
d) de l'eau,
dans lequel les composants (a) à (c) sont présents en une quantité de tous les composants secs de la composition de primaire.

12. Substrat de support revêtu de la revendication 11, dans lequel le substrat de support est un substrat de support en décalage lisse et non poreux.

13. Substrat de support revêtu de la revendication 11, dans lequel les nanoparticules d'amidon sont des nanoparticules d'amidon réticulé, et dans lequel l'alcool de polyvinyle, des nanoparticules d'amidon, la dispersion de latex polymère, la cire et le sel cationique représentent au moins 80% en poids de tous les composants secs de la couche de primaire.
